

## UNITED STATES PATENT OFFICE

1,940,551

PROCESS FOR PRODUCING FAST TINTS  
ON WOOLAlbert Landolt, Basel, Switzerland, assignor to  
the firm of Society of Chemical Industry in  
Basle, Basel, SwitzerlandNo Drawing. Application April 19, 1929, Serial  
No. 356,620, and in Switzerland April 29,  
1928

6 Claims. (Cl. 8—5)

The present invention relates to a new process for producing fast red tints on wool. It comprises the new process and the material that has been dyed according to the new process.

Hitherto it has not been described how with unsulfonated arylides of the 2:3-hydroxynaphthoic acid and unsulfonated diazo-compounds strong dyeings can be produced which are in fact fast to rubbing, light, fulling and potting.

I have found that this result can be attained by treating wool, on the one hand, with the arylide in such grounding baths which contain in the total at least 1 gram of sodium hydroxide per liter of the grounding liquor, and by using, on the other hand, arylides of the 2:3-hydroxynaphthoic acid which derive from such aromatic amines which, apart from one or two  $\text{NH}_2$ -groups, contain no other groups capable of coupling (such as  $\text{OH}$ ,  $\text{N}=\text{CH}_2$ ,  $\text{NH-aryl}$ , etc.) Particularly useful are those arylides which derive from aniline, or also from the halogeno-toluidines.

The above mentioned treatment of the wool does not consist in only a very short padding or impregnation, as is usual for cotton, but the treatment must last sufficiently long to allow the greatest part of the arylide to rush on to the wool. It is appropriate to regulate the temperature of the bath during this treatment in such a manner that the affinity of the arylide for the wool is favorable. As diazo-compounds there come into consideration quite generally the non-sulfonated diazo-compounds of the benzene series, such for instance as the chloro- and bromo-toluidines. The dyeings are characterized not only by their excellent properties of fastness but also by their vividness.

If too little caustic alkali is used there are obtained only feebly colored dyeings which are not fast. Good results are obtained for example with 1.3 to 1.5 grams total  $\text{NaOH}$  in the liter of grounding liquor, or with the alkali concentrations which are usual in dyeing wool with vat-dyestuffs.

As an example of the invention the following directions for dyeing may be given.—

*Grounding.*—The wool is grounded in the bath ratio of 1:30 for  $\frac{3}{4}$  hour at 45° C. in the following bath:

|                                                                        |       |          |    |
|------------------------------------------------------------------------|-------|----------|----|
| 2:3-hydroxynaphthoic acid arylide calculated on the weight of the wool | 1.5—3 | per cent | 50 |
| Turkey red oil                                                         | 5     | cc.      |    |
| Caustic soda solution of 30 per cent strength by weight                | 3.4   | cc.      | 55 |
| Sulfite cellulose waste liquor or glue                                 | 20    | cc.      |    |
| Common salt                                                            | 20    | grams    |    |

are dissolved in water to produce 1000 cc. 60

*Development*

The centrifuged or rinsed wool is developed without intermediate treatment in a cold bath containing per liter 0.01—0.02 mol. of diazotized amine. 65

The dyeings on wool obtained according to these directions are very full, clear and fast.

The following table shows some of the tints which can be obtained in accordance with the invention:

| Arylide                                               | Diazotizing component | Color of the dyeing |    |
|-------------------------------------------------------|-----------------------|---------------------|----|
| Anilide of 2:3-hydroxy naphthoic acid.                | 5-chloro-2-toluidine  | Scarlet.            | 75 |
| Do                                                    | 6-chloro-2-toluidine  | Yellow-red.         |    |
| 5-chloro-2-toluidine of 2:3-hydroxynaphthoic acid.    | 5-chloro-2-toluidine  | Red.                |    |
| Do                                                    | 4-chloro-2-toluidine  | Do.                 |    |
| Do                                                    | 6-chloro-2-toluidine  | Do.                 |    |
| $\alpha$ -naphthylamide of 2:3-hydroxynaphthoic acid. | Meta-xylidine         | Do.                 | 80 |
| $\beta$ -naphthylamide of 2:3-hydroxynaphthoic acid.  | Ortho-anisidine       | Do.                 |    |

What I claim is:—

1. A process for producing fast tints on wool by means of unsulfonated diazo-compounds of the benzene series, and unsulfonated arylides of 2:3-hydroxynaphthoic acid deriving from such aromatic amines which, besides one or two  $\text{NH}_2$  90

- groups, contain no other groups capable of coupling, characterized by causing the arylides to rush on to the wool from such baths which contain at least 1 gram of sodium hydroxide in the liter, and then developing the arylides with the diazo-compounds.

2. A process for producing fast tints on wool by means of unsulfonated diazo-compounds of the benzene series, and unsulfonated arylides of 2:3-hydroxynaphthoic acid deriving from such aromatic amines which, besides one or two  $\text{NH}_2$  groups, contain no other groups capable of coupling, characterized by causing the arylides to rush on to the wool from such baths which contain at least 1 gram of sodium hydroxide in the liter and containing 1.5 to 3 per cent. of the arylide calculated on the weight of the wool, and then developing the arylides with the diazo-compounds.

10 3. A process for producing fast tints on wool by means of unsulfonated diazo-compounds of the benzene series, and unsulfonated arylides of 2:3-hydroxynaphthoic acid deriving from aromatic mononuclear monoamines which, besides one or two  $\text{NH}_2$  groups, contain no other groups capable of coupling, characterized by causing the arylides to rush on to the wool from such baths which contain at least 1 gram of sodium hydroxide in the liter, and then developing the arylides with the diazo-compounds.

15 4. A process for producing fast tints on wool by means of unsulfonated diazo-compounds of the benzene series, and unsulfonated arylides of 2:3-hydroxynaphthoic acid deriving from aromatic mononuclear monoamines which, besides one or two  $\text{NH}_2$  groups, contain no other groups capable of coupling, characterized by causing the arylides to rush on to the wool from such baths the alkalinity of which corresponds to about 1.3 to 1.5 grams of sodium hydroxide in the liter, and containing 1.5 to 3 per cent. of the arylide calculated on the weight of the wool, and then developing the arylides with the diazo-compounds.

20 5. A process for producing fast tints on wool by means of unsulfonated diazo-compounds of the benzene series, and unsulfonated arylides of 2:3-hydroxynaphthoic acid deriving from aromatic mononuclear monoamines which, besides one or two  $\text{NH}_2$  groups, contain no other groups capable of coupling, characterized by causing the arylides to rush on to the wool from such baths the alkalinity of which corresponds to about 1.3 to 1.5 grams of sodium hydroxide in the liter and containing 1.5 to 3 per cent. of the arylide calculated on the weight of the wool, and then developing the arylides with the diazo-compounds.

25 6. A process for producing fast tints on wool by means of unsulfonated diazotized halogenated  $\alpha$ -toluidines, and unsulfonated arylides of 2:3-hydroxynaphthoic acid deriving from aromatic mononuclear monoamines which, besides one or two  $\text{NH}_2$  groups, contain no other groups capable of coupling, characterized by causing the arylides to rush on to the wool from such baths the alkalinity of which corresponds to about 1.3 to 1.5 grams of sodium hydroxide in the liter and containing 1.5 to 3 per cent. of the arylide calculated on the weight of the wool, and then developing the arylides with the diazo compounds.

30 ALBERT LANDOLT. 110

35

40

45

50

55

60

65

70

75

80

85

90

95

100

105

110

115

120

125

130

135

140

145

150